

# United States Patent [19]

Gondo et al.

[11] 3,912,549

[45] Oct. 14, 1975

[54] **METHOD FOR MANUFACTURING A STEEL FOR ENAMELING**

3,183,078 5/1965 Ohtake et al. .... 75/49  
3,806,376 4/1974 Toda et al. .... 148/12.3

[75] Inventors: **Hisashi Gondo; Hiroshi Takechi; Mitsunobu Abe; Kazuo Namba, all of Kisarazu, Japan**

## OTHER PUBLICATIONS

Dewsnap, R. F.; An Investigation of the Rapid Annealing of Sheet Gauge Mild Steel; Special Report 79; pp. 112-120; The Iron and Steel Inst., London, 1963.

[73] Assignee: **Nippon Steel Corporation, Tokyo, Japan**

[22] Filed: **June 28, 1973**

Primary Examiner—W. Stallard

[21] Appl. No.: **374,390**

Attorney, Agent, or Firm—Watson Leavenworth  
Kelton & Taggart

### [30] Foreign Application Priority Data

June 30, 1972 Japan ..... 47-65752

[52] U.S. Cl. .... **148/12 C; 148/12.3**

[51] Int. Cl.<sup>2</sup> .... **C21D 9/46**

[58] Field of Search ..... 148/12, 12.3

### [56] References Cited

#### UNITED STATES PATENTS

2,878,151 3/1959 Beall et al. .... 148/12

### [57] ABSTRACT

The material is a low-carbon steel having not more than 0.25% by weight of Mn, with the particular relation of Mn, S and O content. It is hot rolled and coiled at 600°C to 800°C. It is then cold rolled and annealed for recrystallization. A product having excellent press formability and availability for enameling is thus obtained.

5 Claims, 1 Drawing Figure





**METHOD FOR MANUFACTURING A STEEL FOR  
ENAMELING**

**BACKGROUND OF THE INVENTION**

It has heretofore been required that the cold-rolled steel for enameling having wide applications in various household wares, sanitary articles electric products and so on should have excellent enameling characteristic and press formability.

The availability for enameling can be judged as "fish scaling," "bubbling," "sagging," "boiling," which may be caused after enameling. The fish scaling is caused by the hydrogen entrained in the steel sheet during enameling which is diffused over the surface of the sheet as the time elapses, then breaks the film of the enamel and escapes in the air. In this connection, it has been reported that if there are more voids present inside the steel sheet, the fish scaling less occurs since there are more rooms for the hydrogen to remain.

The most common method to form such voids is to deteriorate the purity of the sheet itself. In other words, it is to increase the non-metallic inclusions therein so as to utilize the voids occurring in the cold rolling of the steel sheet due to the difference in deformability between the inclusions and the others.

This method is, however, undesirable since the fish scaling properties may be improved thereby but the press formability is degraded.

Another effort has been made, wherein the amount of carbon is at first increased in the steel sheet and the massive carbide aggregates are formed before the cold rolling step, said aggregates having same function as the non-metallic inclusions and thus forming voids, and thereafter decarburization is effected instead of using the non-metallic inclusions. However, this method has also disadvantages that the cost for the decarburization and annealing step is too much expensive and that the method itself is not suitable to such material having a great thickness as the bath tub.

The bubbling and the sagging are both the phenomena resulting from the amount of carbon in the steel sheet. Thus, in the former case, the CO or CO<sub>2</sub> gases are generated therefrom, while in the latter case, it is considered to be caused by the fact that due to the lowering of the transformation temperature, the transformation may easily be generated, which results in expansion or contraction of the volume of the material. Accordingly, it is more preferable to have smaller amount of carbon in the material, although it has been reported that it does not raise much problem in a two-coat enameling process.

It is therefore an object of this invention to overcome the defects which would be encountered in the prior art.

It is another object of this invention to control the amount of Mn, S, O to be included in the steel sheet whereby the press formability of the material is remarkably improved.

It is still another object of this invention to control the hot rolling conditions before the cold rolling whereby the material as the steel sheet for porcelain enamel is enhanced with respect to the fish scaling.

**SUMMARY OF THE INVENTION**

This invention relates to a method for manufacturing a steel for enameling.

According to this invention, there is provided a method for the manufacture of a cold-rolled low-carbon steel sheet used for porcelain enamel having excellent press formability and availability for enameling which comprising; providing a low carbon steel material having not more than 0.25% by weight of manganese; said steel material containing Mn, O, and S in the relation of

10

$$-0.20 \leq [Mn\%] - \frac{AW \text{ of Mn}}{AW \text{ of O}} \times [O\%] - \frac{AW \text{ of Mn}}{AW \text{ of S}} \times [S\%] \leq 0.20$$

15

where AW = atomic weight; subjecting said steel material to hot rolling followed by coiling the same at 600°C to 800°C; subjecting said coiled hot rolled strip to cold rolling to thereby obtain a cold rolled strip; and thereafter subjecting said cold rolled strip to recrystallization annealing such as box annealing with over-aging treatment.

The starting material used in this invention is a low-carbon steel having low Mn content. The thin steel sheet to be subjected to press working usually contains

more than about 0.30% Mn. However, an excess amount of Mn exerts an effect upon the mechanical properties of the steel sheet, and in case of the rimmed steel sheet having low-carbon content, it is a common practice to maintain the Mn content as low as possible so as to obtain good surface qualities. The inventors have now found that an appropriate amount of MnS and MnO which is assured by a low Mn content is useful for a continuous annealing treatment. In other words, the amount of Mn required in this invention is

that necessary to fully fix the harmful S and O which exists as impurities due to the high-temperature coiling of the hot rolled sheet described later. That is, the amount by weight of Mn in the steel may be the chemical equivalent to combine with S and O, or slightly

more than that, and it should be not more than 0.25% and preferably 0.20% or less. Also as to the contents of Mn, S and O, it is necessary that K of the following equation lies in the range of  $-0.20 \leq K \leq 0.2$ , and preferably  $-0.15 \leq K \leq 0.15$  particularly when the

prominent effect of this invention is required. It has further been found that the optimum range of K should be  $-0.15$  to  $0$  when the excellent enameling characteristic is particularly required.

55

$$K = [Mn\%] - \frac{AW \text{ of Mn}}{AW \text{ of O}} \times [O\%] - \frac{AW \text{ of Mn}}{AW \text{ of S}} \times [S\%] =$$

60

$$[Mn\%] - \frac{55}{16} \times [O\%] - \frac{55}{32} \times [S\%]$$

If the K is in this range, the average plastic strain ratio, (F value), which shows the press formability and deep drawability of the steel sheet becomes 1.4 or more as seen from the drawing. It is thus obvious that the

steel sheet has extremely good press formability and deep drawability. In passing, it is well known that  $r$  value depends upon the texture.

If Mn exists in an amount of 0.3% or more as in the conventional steel sheet, it forms an excessive MnS and MnO even if the equation  $-0.20 \leq K \leq 0.20$  is satisfied with respect to S% and O%, and exerts an adverse effect upon the properties of the steel sheet. This invention has a feature that the relation of Mn, S and O is within the particular range as mentioned above, but it also has a feature that after hot rolling, the hot rolled steel sheet is coiled at high temperature for the purpose of converting the harmful S and O into the innocent inclusion in the steel having the particular component range as defined above. The existence of S and O in the steel gives rise to red shortness as well as restriction of growth of crystal when the annealing for recrystallization is conducted. Thus, at the time of annealing, a lot of crystal nuclei occurs due to the S inclusion consisting mainly of FeS, which nuclei mutually prevent the growth of crystal grains and at the same time the S inclusion consisting mainly of FeS itself becomes an obstacle to the grain growth. The O gives, as S does, an undesirable factor to the growth of crystal and thus, by means of fixing these harmful S and O with Mn to the condition which is harmless to the grain growth, it is possible to create the circumstances wherein the S and O are dispersed less densely and the full growth of crystal can be expected.

As set forth herein above, this invention is intended to convert the harmful S and O to the harmless MnS and MnO by means of coiling the hot rolled steel sheet at high temperature, which will make it possible to suppress the occurrence of the nuclei at the recrystallization annealing so that the circumstances which are favorable for growth of crystal may be obtained; to accelerate the growth of the crystal grains by means of the self-annealing action of the hot rolled coil during the cooling course; and thereby to lessen the strain energy after cold rolling and preferentially enlarge the crystal having orientation capable of increasing the  $\bar{r}$  value at the recrystallization annealing. This is not described in this specification but can be confirmed by measurement by X-ray of the texture. In order to obtain such desirable result, the coiling temperature as mentioned above should be at least 600°C, and preferably at least 650°C. However, when the coiling is conducted at extremely high temperature, the difference in temperatures of the hot rolled sheet itself is so severe that the control thereof may become difficult. Thus it should be 800°C or less and the preferable range is between 650°C and 800°C.

On the other hand, by means of providing the high coiling temperature at the hot rolling, it also makes it possible to make the carbides in the agglomeration, globular form. The MnS, MnO carbides thus formed may offer an optimum room for making voids at the time of cold rolling, whereby the fish scaling of the steel sheet is considered to be prevented.

#### BRIEF DESCRIPTION OF THE DRAWING

Attached drawing is a diagram showing the relation of the component ratio of the steel sheet with the average plastic strain ratio ( $\bar{r}$ ) and the occurrence ratio of the fish scaling.

Seeing from the drawing, it is understood that the occurrence ratio of the fish scaling depends strongly upon

the K and the coiling temperature. If the coiling temperature is at least 670°C and the K is within the range between -0.2 and 0.2, the occurrence ratio of the fish scaling can be made zero. The K within this range accords with the range in which the  $\bar{r}$  value is at least 1.4, which shows that it is the preferable range both for press formability and for availability to enameling.

The occurrence ratio of the fish scaling in the drawing is obtained by enameling 50 specimens each having a size of 10cm × 10cm, subjecting the same again to the heat treatment at 400°C for 30 minutes and comparing the number of the specimens in which the fish scaling has occurred with others. Even in case of the steel having K of the range in which the occurrence ratio of fish scaling is zero in drawing, the fish scaling properties become much better or occur less often as the K becomes smaller when another more rigid test for judging the fish scaling properties is conducted. That is, when the hydrogen gas is compulsorily generated on one side of the sheet and the time for the hydrogen gas to reach the reverse side of the sheet (the hydrogen pass time) is measured for judging the fish scaling properties, it is found that as the K becomes smaller the hydrogen pass time becomes longer, and when the K changes from plus to minus the hydrogen pass time becomes remarkably longer.

Generally, the more voids which are sources for absorbing hydrogen, the longer hydrogen pass time.

Thus, it can be further said that the longer the hydrogen pass time is, the better are the fish scaling properties. The reason why the fish scaling properties become remarkably better particularly in the range of K being minus may be that the amount of MnS and MnO is increased within the range that they do not harm the properties of the material, which result in prominent generation of voids due to the cold rolling.

The specimens in the drawing are manufactured as follows:

A rimmed steel material having composition of C: 0.03 to 0.05%, Mn: 0.14 to 0.31%, S: 0.007 to 0.022%, O: 0.010 to 0.085%, the rest: substantially Fe is hot rolled, coiled at 700°C to 730°C, and then cold rolled to the final thickness (0.8mm). The resulting steel sheet is subjected to the continuous annealing treatment for 700°C × 1.5 minutes and then to the over-aging treatment for 350°C × 5 minutes.

The advantage of the present invention can also be confirmed by using the box annealing (700°C × 4 hours) after cold rolling and similar preferable results can be obtained.

The steel material to which the present invention may be applied is generally one which is produced by converter or other steel manufacturing furnaces, and subjected to the steps of casting, blooming, hot-rolling, etc. and further, cold rolling, continuous annealing including over-aging or box annealing and, if desired, the temper rolling treatment.

The conditions for those steps may vary as desired in so far as the requirements such as component of the material or the coiling temperature for the hot rolled sheet, etc., are observed.

The amount of C for the present invention may be that contained in the ordinary low carbon cold rolled steel sheet. If it is desired to obtain lower carbon content for pursuing more excellent press formability, or lower bubbling or sagging, the molten steel may be degassed under vacuum conditions or the material may be

subjected to decarburization treatment at the time of annealing, whereby the above object can easily be accomplished.

In the present invention, it is advantageous to keep the N content in the sheet as low as possible, whereby the stabilization of the *r* value, the decrease of the strain aging property as well as the excellent press formability can be obtained. As for the strain aging property, it is possible to add such N-fixing elements as Al, B, V and the like.

#### DESCRIPTION OF THE PREFERRED EMBODIMENT

A steel sheet obtained by converter and subjected to the usual steps of casting, blooming and hot rolling was 15 coiled at 700°C to 730°C to obtain a hot rolled coil, which was then allowed to stand in the air to the ordinary temperature. This hot rolled sheet was further subjected to the cold rolling step to obtain the final thickness of 0.7mm. Thereafter the recrystallization annealing for 700°C × 1 minute and the subsequent over-aging treatment for 350°C × 2 minutes were effected in the continuous annealing system and further the temper rolling was effected to the extent of 1 to 1.5%. The table below shows the chemical compositions of the 20 materials (a) and (b) of the invention (analysis of the product) and the properties of the steel sheet obtained. By way of comparison, the data of the steel plate having a large *K* value are also shown in the table.

As is obvious from the above table, the steel sheet obtained by the present invention has excellent properties as compared with that obtained by the prior art.

We claim:

5 1. A method for the manufacture of a cold-rolled low-carbon steel sheet used for porcelain enamel having excellent press formability and suitability for enameling which comprises: providing a low carbon steel material having not more than 0.25% by weight of manganese; said steel material containing Mn, O and S in the relation of

$$-0.20 \leq [Mn\%] - \frac{AW \text{ of } Mn}{AW \text{ of } O} \times [O\%] - \frac{AW \text{ of } Mn}{AW \text{ of } S} \times [S\%] \leq 0$$

where AW — atomic weight; subjecting said steel material to hot rolling followed by coiling the same at 600°C to 800°C; subjecting said coiled hot rolled strip to cold rolling to thereby obtain a cold rolled strip; and thereafter subjecting said cold rolled strip to recrystallization annealing.

|                                                   | The material of this invention<br>(0.7mm thick) |                             | The material<br>to be com-<br>pared<br>(0.7mm thick) |
|---------------------------------------------------|-------------------------------------------------|-----------------------------|------------------------------------------------------|
|                                                   | (a)                                             | (b)                         |                                                      |
| Composition                                       |                                                 |                             |                                                      |
| C %                                               | 0.04                                            | 0.04                        | 0.04                                                 |
| Mn                                                | 0.18                                            | 0.17                        | 0.33                                                 |
| S                                                 | 0.010                                           | 0.015                       | 0.010                                                |
| O                                                 | 0.042                                           | 0.075                       | 0.028                                                |
| K                                                 | 0.02                                            | -0.11                       | 0.22                                                 |
| Coiling temperature °C                            | 700 to 720                                      | 670 to 680                  | 530 to 550                                           |
| Annealing (Continuous conditions)                 | 700°C×1min.<br>+350°C×2min.                     | 700°C×1min.<br>+350°C×2min. | 700°C×1min.<br>+350°C×2min.                          |
| Temper rolling(%)                                 | 1.0 to 1.5                                      | 1.0 to 1.5                  | 1.0 to 1.5                                           |
| a) After temper rolling:                          |                                                 |                             |                                                      |
| Yield point (kg/mm²)                              | 19.1                                            | 19.5                        | 22.1                                                 |
| Tensile strength (kg/mm²)                         | 31.8                                            | 32.0                        | 34.7                                                 |
| Elongation (%)                                    | 45                                              | 44                          | 42                                                   |
| <i>r</i>                                          | 1.60                                            | 1.5                         | 1.12                                                 |
| C C V (mm)                                        | 26.02                                           | 26.25                       | 27.21                                                |
| Erichsen test (mm)                                | 10.8                                            | 10.8                        | 10.3                                                 |
| Elongation at yield point (%)                     | 0                                               | 0                           | 0                                                    |
| b) After aging:                                   |                                                 |                             |                                                      |
| Elongation at yield point (%) (100°C×60 min.)     | 3.1                                             | 3.0                         | 5.6                                                  |
| Elongation at yield point (%) (room temp. ×3days) | 0                                               | 0                           | 1.2                                                  |
| Occurrence ratio of fish scaling after enameling  | 0%                                              | 0%                          | 4.2%                                                 |
| Hydrogen pass time (25°C)                         | 72                                              | 135                         | 15                                                   |

$$\text{Remarks } K = [Mn\%] - \frac{AW \text{ of } Mn}{AW \text{ of } O} \times [O\%] - \frac{AW \text{ of } Mn}{AW \text{ of } S} \times [S\%]$$

2. A method for the manufacture of a cold-rolled low-carbon steel sheet used for porcelain enamel having excellent press formability and suitability for enameling which comprises: providing a low carbon steel material having not more than 0.25% by weight of manganese; said steel material containing Mn, O, and S in the relation of

$$-0.15 \leq [Mn\%] - \frac{AW \text{ of } Mn}{AW \text{ of } O} \times [O\%] - \frac{AW \text{ of } Mn}{AW \text{ of } S} \times [S\%] \leq 0$$

where AW — atomic weight; subjecting said steel material to hot rolling followed by coiling the same at

600°C to 800°C; subjecting said coiled hot rolled strip to cold rolling to thereby obtain a cold rolled strip; and thereafter subjecting said cold rolled strip to recrystallization annealing.

5 3. A method according to claim 2 in which said material has not more than 0.20% by weight of manganese.

4. A method according to claim 2 in which said recrystallization annealing is a continuous annealing 10 with over-aging treatment.

5. A method according to claim 2 in which said recrystallization annealing is a box annealing.

\* \* \* \* \*

15

20

25

30

35

40

45

50

55

60

65

UNITED STATES PATENT OFFICE  
CERTIFICATE OF CORRECTION

PATENT NO. : 3,912,549

DATED : October 14, 1975

INVENTOR(S) : Hisashi Gondo et al

It is certified that error appears in the above-identified patent and that said Letters Patent are hereby corrected as shown below:

At Col 2, line 25, "box annealing with over-aging"  
should read --box annealing or continuous annealing with  
over-aging--.

At Col. 3, line 2, "r value" should read --r value--.

Signed and Sealed this

Thirtieth Day of January 1979

[SEAL]

Attest:

RUTH C. MASON  
Attesting Officer

DONALD W. BANNER  
Commissioner of Patents and Trademarks